

## UNITED STATES PATENT OFFICE.

JOSEPH E. BABB, OF PITTSBURGH, PENNSYLVANIA, ASSIGNOR TO WAVERLY OIL WORKS COMPANY, OF PITTSBURGH, PENNSYLVANIA, A CORPORATION OF PENNSYLVANIA.

## FUEL MIXTURE FOR INTERNAL-COMBUSTION ENGINES.

No Drawing.

Application filed April 22, 1925. Serial No. 25,136.

To all whom it may concern:

Be it known that I, JOSEPH E. BABB, a citizen of the United States, and a resident of Pittsburgh, in the county of Allegheny and State of Pennsylvania, have invented a new and useful Improvement in Fuel Mixtures for Internal-Combustion Engines; and I do hereby declare the following to be a full, clear, and exact description thereof.

My invention relates to a mixture that may be added to the usual fuels of internal combustion engines for the purpose of effecting more uniform compression and for permitting increased compression in the engine cylinders without producing "knocking."

Heretofore it has been proposed to add to gasoline and like motor fuels lead compositions that are soluble in gasoline and the like, to increase the effectiveness of such fuel. One objection to these mixtures arises from the fact that metallic lead is liberated by the explosion in the engine cylinder and this liberated lead collects upon the sparking contacts and elsewhere in the engine and the exhaust line, interfering with the proper operation of the engine. These lead mixtures have been designated in my copending applications, Serial No. 756,071, filed December 15, 1924, and Serial No. 9,301, filed February 14, 1925, as lead soap and may consist of rosin oil, which is a distillation product of rosin, and an oxide of lead such as litharge, or the like.

One object of my invention is to provide a mixture wherein an acid-carrying compound is employed in connection with the soap mixture or in the fuel to which the soap is added, for the purpose of rendering the lead volatile or gaseous upon explosion in the cylinder, so that it will be carried off through the exhaust, and thereby be prevented from accumulating in the engine cylinder.

Another object of my invention is to improve generally the effectiveness of fuel mixtures employed in internal combustion engines and the like.

In order to enable my invention to be more clearly understood, I will describe one of the lead soap mixtures with which my acid-carrying element may be employed, it being understood that such a carrier may be used

in other fuel mixtures with satisfactory results.

One composition which may be employed to increase the effectiveness of gasoline, benzol and the like, comprises a soap composed of 100 parts rosin oil and 15 parts litharge. The litharge combines with the acids of the rosin oil and forms what is known as lead rosin oil soap. To 100 parts of this soap 55 50 parts of free oleic acid, or red oil is added. This mixture is somewhat viscous and may be diluted with a solvent such as zero paraffine oil, kerosene, benzol, xylol, or the like, one of which may be added to the soap in a quantity substantially equal to the quantity of oleic acid employed. The foregoing mixture is added to the main body of 60 the motor fuel, preferably in such quantity that the proportion of the lead to the fuel is approximately as 1 to 1000.

While the fuel to which lead has been added, as stated, permits of increased pressure in the engine cylinder without causing knocks, the explosion of such mixture results in the liberation of metallic lead. Unless this lead is removed, it will foul the 70 75 80 85 90 95 100 sparking contacts as above explained. Heretofore, halogen carriers such as carbon tetrachloride have been employed for effecting volatilization of the liberated lead, so that it would be carried away with the exhaust gases. I have discovered that if an acid carrying compound such as nitrobenzol (commonly known also as oil of mirbane) is mixed with the fuel into which the lead mixture is introduced, in quantities sufficient to chemically unite with the lead present after an explosion in the engine cylinder, the liberated lead will be rendered volatile or gaseous and be carried off with the exhaust gases of the engine. The nitrobenzol may be introduced into the main body of the fuel either before the lead soap composition is placed therein or afterwards.

I prefer to use an acid carrying compound such as nitrobenzol because it has a greater affinity for the lead than do the various halogen carriers heretofore employed, and therefore more effectively volatilizes the liberated lead. One mixture which I have found to be effective in the volatilization of the lead liberated by the explosions in the

motor consists of 39.44% rosin oil, 5.917% PbO, 25.6+% oleic acid, 22.419% xylol, 6.57% nitrobenzol. This mixture when exposed over night to a temperature from 10° to 15° F. does not show a precipitate.

The nitrobenzol may also be employed in various other mixtures, such for instance as those wherein solvents such as kerosene, benzol or zero paraffine oil are substituted for 10 the zero paraffine oil, but these latter mixtures may show precipitation upon exposure to low temperatures, although such precipitation will again be taken up in solution when the temperature rises.

15. Also, I do not limit myself to the employment of nitrobenzol as a volatilizing agent, but may use instead thereof an organic acid carrying compound such as ethyl sulphate or methyl sulphate, or any acid 20 organic compounds of nitric acid or sulphuric acid that are soluble or miscible in hydrocarbon fuels.

I claim as my invention:

1. In a fuel mixture for internal combustion engines, the combination with a lead oxide, of an organic acid compound in quantity sufficient to chemically unite with the lead present after combustion, for rendering

substantially all of the lead volatile or gaseous.

2. An explosive fuel mixture comprising 39.44% rosin oil, 5.917% PbO, 25.6+% oleic acid, 22.419% xylol, 6.57% nitrobenzene.

3. In a fuel mixture for internal combustion engines, the combination with a distillation product of rosin and a lead oxide, of nitrobenzene in quantity sufficient to volatilize the lead liberated upon explosion of the mixture.

4. In a fuel mixture for internal combustion engines, the combination with a distillation product of rosin and a lead oxide, of an organic acid carrying compound in quantity sufficient to volatilize the lead 45 which is liberated upon explosion of the mixture.

5. In a fuel mixture for internal combustion engines, the combination with a hydrocarbon fuel having a lead oxide, of nitrobenzene in sufficient quantity in order to chemically unite with the lead present after combustion, for rendering the lead volatile.

In testimony whereof I, the said JOSEPH E. BABB, have hereunto set my hand.

JOSEPH E. BABB.